

# United States Patent

[19]

Conner

[11] 3,915,631

[45] Oct. 28, 1975

[54] **PROCESSES TO MAKE OLIVE DRAB TO GREENISH-GOLD MINERAL DYE SHADES FOR CELLULOSICS**

[75] Inventor: **Charles J. Conner**, Matairie, La.

[73] Assignee: **The United States of America as represented by the Secretary of Agriculture**, Washington, D.C.

[22] Filed: **June 28, 1973**

[21] Appl. No.: **374,585**

[52] U.S. Cl. .... **8/52; 8/54.2; 252/8.6**

[51] Int. Cl.<sup>2</sup> .... **C09B 61/100; D06P 1/00; D06P 3/60; D06M 00/00**

[58] **Field of Search**..... **8/52; 252/8.6**

[56] **References Cited**

UNITED STATES PATENTS

1,686,540 10/1928 White ..... 8/52  
2,091,539 8/1937 White ..... 8/52

2,923,592 2/1960 Crosland ..... 8/52  
3,794,466 2/1974 Conner ..... 8/52

*Primary Examiner*—Benjamin R. Padgett

*Assistant Examiner*—Donald P. Walsh

*Attorney, Agent, or Firm*—M. Howard Silverstein; Max D. Hensley

[57] **ABSTRACT**

Olive drab to greenish-gold mineral dye shades are imparted to cellulosic textiles by a two-solution aqueous process wherein critical proportions of ferrous salts and chromic chloride are mixed in a first aqueous solution, applied to the textile and dried, then a mixture of sodium hydroxide and sodium carbonate are applied in a second aqueous solution, and the color developed upon the drying-curing step. The coloration is controllably olive drab when the ferrous salt content is low and controllably greenish-gold when the ferrous salt content is high.

**4 Claims, No Drawings**

**PROCESSES TO MAKE OLIVE DRAB TO  
GREENISH-GOLD MINERAL DYE SHADES FOR  
CELLULOSICS**

A non-exclusive, irrevocable, royalty-free license in the invention herein described throughout the world for all purposes of the United States Government, with the power to grant sublicenses for such purposes, is hereby granted to the Government of the United States of America.

The prior art shows that mineral colors are produced by treating cellulosics with metal salts in aqueous solution, followed by treatment with an alkali to produce the metal hydroxide or hydrated oxide in the cellulosic (as pigment), resulting in colored-mineral dyeings. These colors are simple "double decomposition" reaction products, and are well known in the trade. However, when a ferrous salt is incorporated into a chromic chloride solution, the ferrous salt is capable of producing basic ferroso-ferric hydrated oxides through partial oxidation and heating with excess concentrated alkalies. Since our processing can be demonstrated to be a series of reactions, over and above simple double decomposition, it is unique and novel in the field of mineral dyeings, offering several new and attractive color shades for stable textile-mineral dyeing.

The present invention consists of treating an aqueous solution of chromic chloride with ferrous salt (sulphate), to produce an aqueous bath of chromic chloride and ferrous 120°-130°C, the intimate chromic chloride and ferrous sulphate salts are deposited and dried in the cellulosic, producing a "pure dark green" color shade. The treated cellulosic is then wetted in the alkali bath, the excess alkali liquor removed by squeezing, and the wet alkali-treated cellulosic subjected to 150°-155°C for 2 to 3 minutes. At the end of this time, the color changes from "pure green" to a "golden" or "yellow-brown" shade. Heating in contact with the excess alkali produces this change at about 150°C. The dyed cellulosic is then hot water washed to remove soluble matter, and dried at 130°-150°C for 2 to 3 minutes. The mineral dyeing is uniform and colored in the "olive drab to greenish-gold" range, depending on the ratio of ferrous salt to chromium in the first bath.

The main object of the invention is to provide a unique process for dyeing "olive drab to greenish-gold" mineral dye shades on cellulosics, using low cost chemicals and conventional mill equipment, to produce highly desirable attractive mineral dye color shades.

A second object of the invention is to use conventional chromic chloride, familiar to most textile finishers, inexpensive and readily available ferrous sulphate, and "alkali" chemicals which are inexpensive and conventionally used in textile mills, for the development of dye shades of very attractive appearance from inexpensive materials, capable of being finished with hydrophobic wax water repellents, as with other conventional mineral dyeings.

Utility of the invention is obviously in the field of mineral dyeings and weatherable goods, such as pigmented (dyed) cellulosics for tents, sails, tarpaulins, umbrellas, awnings, ropes, shoe linings, boat covers, canvas shoes, upholstery, etc.

**SUMMARY**

This invention can best be described as one disclosing specific inorganic chemical formulations and a pro-

cess for imparting to cellulosic textiles durable greenish-yellow (golden) to olive drab coloration through mineral dyeing, the process comprising impregnating a cellulosic textile with an aqueous solution containing ferrous sulphate and liquid 8-9% Cr chromic chloride solution, wherein the ferrous sulphate is about 1.5% to 2.95% of the solution and the chromic chloride content is about from 78% to 79%; drying the wet impregnated textile at about from 120° to 130°C for about 2 to 3

10 minutes; impregnating the textile again, with an aqueous alkali solution containing about 5% to 15% of sodium hydroxide and about from 5% to 25% sodium carbonate; drying-curing the wet impregnated textile at about from 150° to 155°C for about 2 to 3 minutes to develop the color; and hot water-washing at a temperature of about 55°C for about from 2 to 3 minutes to remove residual alkalies; and drying at temperatures about from 130° to 150°C for about 2 to 3 minutes.

The following examples are presented to illustrate the invention and certain aspects of its usefulness. These are not to be interpreted as limiting the invention in any manner whatsoever. The treatments were also applied to paper, wood, and other fabrics having cellulosic compositions.

**EXAMPLE 1**

**(Bath) Olive Drab Mineral Dyeing Procedure For  
Scoured Cotton Duck**

| BATH A |                                                                 |
|--------|-----------------------------------------------------------------|
| 40.0   | grams Chromic Chloride Solution (8%-9% Chromium Metal Content)* |
| 10.0   | grams Water (distilled or soft)                                 |
| 0.8    | gram Ferrous sulphate (heptahydrate) crystals                   |
| 50.8   | grams Bath A (For Olive Drab Dye Shade)                         |

| BATH B |                                               |
|--------|-----------------------------------------------|
| 5.0    | grams Sodium Hydroxide Pellets (Caustic Soda) |
| 15.0   | grams Soda Ash (Sodium Carbonate) Anhydrous   |
| 80.0   | grams Water (distilled or soft)               |
| 100.0  | grams Bath B (Alkali)                         |

\*Industrial chromic chloride is supplied as a liquid with 8% to 9% chromium metal content. 40 grams of this liquid in a 50.8 gram Bath (A) = 78.7% of Bath (A).

**EXAMPLE 2**

**45 Procedure for "Olive Drab" Mineral Dyeing Procedure  
on Cotton Scoured Duck**

A 2×4 inch section of scoured cotton 9 oz. duck was wetted thoroughly in Bath A, the excess squeezed out through rollers, and the wet fabric heated in the oven at 120°-130°C for 2 to 3 minutes, until the dry treated fabric was pure "dark green." The dry fabric was then immersed and thoroughly wetted with Bath B, squeezed free of excess liquid alkali (rollers), and returned to the oven and heated at 150°-155°C for 2 to 3 minutes, until a "golden brown" color was noted in the dyed area. The dyed fabric was then hot tap water (55°C) washed for 3 minutes to remove all soluble salts and alkali, and was then returned to the oven and heated at 130°-150°C for 2 to 3 minutes. The cured and dry fabric was dyed a uniform "Olive Drab."

**EXAMPLE 3**

**Demonstration To Show That The Alkali Must Be  
Present in Curing After Double Decomposition**

Baths A and B were prepared as in Example 1. The scoured duck fabric was wetted, squeezed, and oven dried at 120°-130°C with Bath A. The fabric was then

wetted thoroughly in Bath B, squeezed, and washed free of alkali and salts with hot tap water. The fabric was dyed a grayish-green. It was then oven dried for 2 to 3 minutes at 130°-150°C. A grayish-green mineral dyeing resulted, without the yellowish-green color of "Olive Drab," showing that cure without contact with free alkali did not produce the necessary conversion to "Olive Drab."

## EXAMPLE 4

## (Bath) Greenish-Gold Mineral Dyeing Procedure For Scoured Duck

| BATH A |                                                                 |
|--------|-----------------------------------------------------------------|
| 40.0   | grams Chromic Chloride Solution (8%-9% chromium metal content)* |
| 10.0   | grams Water (Distilled or soft)                                 |
| 1.0    | gram Ferrous Sulphate (heptahydrate crystals)                   |
| 51.0   | grams Bath A (Greenish-Gold)                                    |

| BATH B |                                               |
|--------|-----------------------------------------------|
| 5.0    | grams Sodium Hydroxide Pellets (Caustic Soda) |
| 15.0   | grams Soda Ash (Sodium Carbonate) Anhydrous   |
| 80.0   | grams Water (Distilled or soft)               |
| 100.0  | grams Bath B (Greenish-Gold) Alkali           |

(Note: Both baths should be uniform, clear, solutions)

\*Industrial chromic chloride is supplied as a liquid with 8% to 9% chromium metal content. 40 grams of this liquid in a 51.0 gram Bath (A) = 78% of Bath (A).

## EXAMPLE 5

## Procedure for "Greenish-Gold" Mineral Dyeing on Scoured Duck

A 3×4 inch piece of scoured 9 oz. duck was treated with Bath A according to procedure in Example 2, followed by treatment with Bath B according to procedure in Example 2. Oven heating and washing and drying procedures were the same as in Example 2. A uniform "greenish-gold" mineral dyeing resulted.

## EXAMPLE 6

In Example 1, baths were prepared with the Ferrous Sulphate varied between 0.25 gram and 1.50 gram, with Bath B varied between 5 gms. NaOH and 15 gms. NaOH and soda ash varied between 5 gms. and 25 gms. Variations in the Alkali Bath (B)<sup>†</sup> made no difference in end results, and concentration of the bath can be varied to keep an excess alkali in the bath. Where the Ferrous Sulphate was varied, the following color shades were obtained:

- 0.25 gm. Ferrous Sulphate—Green mineral dyeing
- 0.50 gm. Ferrous Sulphate—Bright medium green
- 0.80 gm. Ferrous Sulphate—Olive Drab shade
- 1.00 gm. Ferrous Sulphate—Greenish-Gold dye shade
- 1.50 gm. Ferrous Sulphate—Brown(greenish) dye shade

In Bath A, (of Example 6), all other components

(other than Ferrous Sulphate) remain constant, per Example 1. Applications were made with 9 oz. scoured cotton army duck in each evaluation.

† With 5 gms. NaOH and 5 gms. Na<sub>2</sub>CO<sub>3</sub>, the water content is 90%  
With 15 gms. NaOH and 25 gms. Na<sub>2</sub>CO<sub>3</sub>, the water content is 60% } range  
% H<sub>2</sub>O in Bath (B)

## EXAMPLE 7

10 Some of the dyed swatches were treated with a 7% parrafin-ammonium stearate wax water emulsion, followed by oven heating at 145°C/2 minutes. The color shades were slightly deepened, but not changed, and a degree of water repellency was attributed by the wax treatment. In other words, the dyed fabrics may be wax finished according to any commercial conventional wax-finishing procedure, to attribute water repellency characteristics.

## EXAMPLE 8

20 Dyed swatches of both olive drab and greenish gold were exposed to outdoor weathering on wooden frames. After one month, no evidence of color change was noted, and the mineral dyeings were stable to sunlight and weathering.

I claim:

1. A process for imparting to cellulosic textiles durable greenish-yellow (golden) to olive drab coloration through mineral dyeing, the process comprising impregnating a cellulosic textile with an aqueous solution containing ferrous sulphate and liquid 8-9% Cr chromic chloride solution, wherein the ferrous sulphate is about 1.5% to 2.95% of the solution and the chromic chloride solution content is about from 78% to 79%; drying the wet impregnated textile at about from 120° to 130°C for about 2 to 3 minutes; impregnating the textile again, with an aqueous alkali solution containing about 5% to 15% of sodium hydroxide and about from 5% to 25% sodium carbonate; drying-curing the wet impregnated textile at about from 150° to 155°C for about 2 to 3 minutes to develop the color; and hot water-washing at a temperature of about 55°C for about from 2 to 3 minutes to remove residual alkalies; and drying at temperatures about from 130° to 150°C for about 2 to 3 minutes.
2. The process of claim 1 wherein the ferrous sulphate in the first solution is about 1.50% to yield a cellulosic textile with an olive drab coloration.
3. The process of claim 1 wherein the ferrous sulphate in the first solution is about 1.96% to yield a cellulosic textile with a greenish-gold coloration.
4. The process of claim 1 wherein the ferrous sulphate in the first solution is about 2.95% to yield a brownish shade of greenish-gold.

\* \* \* \* \*